

## UNITED STATES PATENT OFFICE

2,402,862

## WELL CASING

Edwin C. Wright, Beaver, Pa., assignor to National  
Tube Company, a corporation of New JerseyNo Drawing. Application March 25, 1943,  
Serial No. 480,551

2 Claims. (Cl. 138—47)

1

The pipe and tubing used as casing for shutting out water in the drilling of wells for the production of oil, and also water wells for irrigation purposes, has to resist high external pressures due to the occurrence of water-bearing strata at considerable elevations above the bottom of the hole. The drilling of oil wells to depths as great as 15,000 ft. has greatly increased the stresses imposed upon casing, especially in such very deep oil wells. It has long been known that the resistance of the casing to external pressure is dependent entirely upon the true elastic limit of the casing material. As soon as the external pressure develops a stress in the casing which exceeds the true elastic limit of the material in the casing, the structure becomes unstable and collapses much like a very long column. As a result, the casing used in oil and water wells has had to develop a true elastic limit of higher and higher values as the depths of the wells increased.

At the present time the API lists four standard grades of casing which are classified according to the yield point of the material. The yield point is proportional to the true elastic limit of the casing. These grades are tabulated below

| Grade | Yield point,<br>p. s. i. |
|-------|--------------------------|
| F-25  | 25,000                   |
| H-40  | 40,000                   |
| J-55  | 55,000                   |
| N-80  | 80,000                   |

The grade of casing employed of any given size is determined by the depth of the hole.

2

containing less than 1% manganese. The latter two grades of casing—namely, J-55 and N-80—require special alloy additions, such as chromium, manganese, molybdenum, or nickel or combinations thereof, to develop the necessary elastic limit to provide the collapse resistance required at great depth. It will thus be evident that a considerable quantity of alloy steel for oil well casing and oil well tubing is necessary for wells 10 below 6,000 ft. deep.

Studies of the physical properties and collapse resistance of thoroughly deoxidized high-phosphorus steels have shown me that adjustments of the carbon, manganese, and phosphorus contents enable the production of deep well casing and tubing which will be adequate for all existing wells drilled. The general composition of these high phosphorus steels, which must be made extremely low in oxygen combined with the 20 iron, is tabulated below:

|               |           |
|---------------|-----------|
| Carbon        | .15—.40   |
| Manganese     | .30—2.00  |
| Phosphorus    | .10—.30   |
| Silicon       | .15—.50   |
| Sulphur       | .05 max.  |
| Oxygen as FeO | Under .02 |
| Iron          | Balance   |

As typical examples of the properties of steels 30 made in this range of composition, Table I shows the tensile strength, yield point, elongation in 2" (ductility), and Charpy impact properties of several steels made with the high phosphorus content and thoroughly deoxidized as to contain less than .02% oxygen as FeO.

Table I

|                  | Steel No. |        |         |         |         |         |         |
|------------------|-----------|--------|---------|---------|---------|---------|---------|
|                  | 1         | 2      | 3       | 4       | 5       | 6       | 7       |
| Carbon           | 0.29      | 0.30   | 0.31    | 0.30    | 0.30    | 0.41    | 0.39    |
| Manganese        | 1.00      | 1.25   | 1.48    | 1.28    | 1.50    | 1.53    | 1.51    |
| Silicon          | .23       | .20    | .21     | .23     | .22     | .21     | .23     |
| Phosphorus       | .18       | .11    | .12     | .21     | .19     | .12     | .20     |
| Sulphur          | .027      | .031   | .028    | .021    | .029    | .022    | .027    |
| Tensile strength | 103,560   | 99,510 | 108,880 | 109,510 | 116,880 | 121,040 | 131,040 |
| Yield strength   | 72,500    | 69,700 | 74,900  | 76,600  | 81,800  | 84,600  | 91,900  |
| Elongation 2"    | 29.2      | 31.0   | 27.6    | 25.2    | 23.4    | 22.0    | 20.8    |
| Charpy impact    | 36.1      | 37.2   | 30.2    | 29.5    | 26.1    | 24.2    | 22.0    |

The first two types of casing—namely, F-25 and H-40—are produced readily from regular open hearth steel or simple analysis, at least

The physical properties given in Table I for the seven different typical compositions show that pipe and tubing of satisfactory ductility, tough-

ness, and yield point can be produced from these types of steel to fit all the present standard grades of casing and tubing used in the drilling of oil wells and water wells. The thorough reduction in the oxygen combined with the iron characterizing these steels enables the production of steel articles of extremely good toughness and ductility which heretofore have not been produced with steel compositions containing considerable amounts of phosphorus. The steel of this composition may be made by the acid Bessemer process, the basic or acid open hearth process, or the basic or acid electric melting process.

I claim:

1. Well casing made of steel containing from .15 to .40% carbon, from .30 to 2.00% manganese, from .10 to .30% phosphorus, from .15 to .50% silicon, not more than .05% sulphur, less than .02% oxygen combined with iron and with the remainder substantially all iron.

2. Well casing made of steel containing sufficient phosphorus to materially enhance the collapse resistance of the casing and less than .02% oxygen combined with its iron.

EDWIN C. WRIGHT.